

## UNITED STATES PATENT OFFICE

2,057,456

## DENTAL IMPRESSION COMPOSITION

Raymond B. Stringfield, Los Angeles, Calif., assignor to Dental Plastics Company, Los Angeles, Calif., a corporation of California

No Drawing. Application July 18, 1933,  
Serial No. 681,004

9 Claims. (Cl. 18—47)

This invention relates to a dental composition and more specifically it relates to a composition of matter to be employed in the preparation of dental impressions.

5 For many dental purposes such as the making of full dentures, partial dentures, bridges, etc. it is necessary for the dentist to be able to accurately reproduce portions of the mouth of the subject. Such reproductions often involve the duplication of undercuts of more or less severity, as for instance in the case where a tooth or teeth have been extracted and the adjacent teeth have crowded together.

10 For many years dental impressions have been taken with materials such as plaster of Paris, or various shellac or wax compositions. These materials have little or no elasticity and while it is not difficult to take some impressions with them, such as for most full dentures, it is not possible to reproduce accurately undercuts without either breaking the impression and re-assembling it as is done with plaster, or taking the impression in sections as is the practice in the use of shellac and wax compounds. The foregoing methods obviously involve time and there is the danger of inaccuracy, as well as discomfort to the patient.

15 By the use of an impression material which may be introduced in the mouth in a fluid or plastic condition and cooled to an elastic state, it is possible to take an impression which will accurately reproduce all details of the portion of the mouth under examination, and which due to its elasticity, can be removed from any undercuts present without losing the accuracy of the impression.

20 Due to the narrow range of temperature which the human mouth can stand, rather strict limitations are placed on the types of elastic materials which can be used. These materials must obviously be either fluid or plastic when they are seated to place in the mouth and must change by cooling to an elastic gel which will permit removal from the undercuts without permanent distortion. They must also either harden to a solid or be a sufficiently tough and rigid gel so that they may be used as molds for models of plaster or other compounds to be poured into them.

25 It is possible by the use of a hydro-colloid to obtain a compound which is a viscous fluid when slightly warmed and which cools at room temperature, or by the use of ice water, to a gel which is elastic enough to reproduce undercuts properly and is also sufficiently firm to withstand a reasonable amount of handling and which can be used.

30 as a mold to receive plaster. The hydro-colloid types of denture materials are objectionable because they require special equipment to insure the correct proportion of water in the mixture, and proper cooling of the impression in the mouth in order to obtain the necessary degree of rigidity or toughness. Furthermore, impressions made from hydro-colloids are relatively fragile and are easily injured when handled. Additionally it is necessary to supply some means for the prevention of the evaporation of water from the impression after it has been removed from the mouth, otherwise a change of shape or size in the impression takes place.

35 The use of non-aqueous gels in the production of dental impressions eliminates most of the objections inherent in other types of impression materials. These non-aqueous gels may be made in various ways. However, I find the most suitable types to be made by the action of metallic soaps, such as aluminum stearate or palmitate, 20 with waxes or pitches such as stearine pitch. Gels produced in this manner become plastic when warmed instead of liquid as do the aqueous gels and may be so compounded that they form an elastic mass at temperatures slightly above the 25 temperature of the mouth (98.6° F.). Thus no special cooling is required in order to obtain the proper degree of rigidity in the impression material. When impressions made using these gels are removed from the mouth and further cooled, 30 they become quite rigid and may be handled without any unusual or special precautions to prevent a change in shape or size.

An ideal dental impression material should 35 have the following characteristics:

1. It must accurately reproduce all details of the impression.
2. It must change from a plastic to an elastic gel at a temperature comfortable to the mouth.
3. It must be workable in the fingers without sticking so that the dentist may properly load a tray.
4. It must not stick to the teeth or gums when the impression is being removed. In some cases 45 the removal of the impression is assisted by the use of a separating medium, such as glycerine or a glycerine jelly which is applied to the teeth prior to taking the impression.
5. It must not have an obnoxious taste or 50 odor, or be injurious to the mouth tissue.
6. It must not decompose appreciably when placed in water to cool.
7. The impression must not change dimen- 55

sions upon standing for several hours at cool room temperatures.

8. The impression should be removable from the plaster model without sticking, although it is feasible at times to aid this property by the use of a thin separating medium, such as alcoholic solutions of sandarac, or other resins, applied to the impression before pouring the plaster.

Most gels produced from waxes and metallic soaps are not tough and are difficult to handle due to their fragility and also because they stick to the plaster cast. I have discovered that these gels may be improved by the substitution of a tougher material for a part, or all, of the waxes.

15 By the substitution of stearine pitch for a part, or all of the wax, it is possible to obtain a gel with metallic soaps which has greatly improved physical characteristics when employed in the production of dental impression compositions.

20 Stearine pitch is a by-product of the stearic acid industry. It is a complex mixture of stearine, stearine acid and other materials. It is black in color due to the carbon formed by decomposition during manufacture. When cooked with a metallic soap, as for example, aluminium stearate or palmitate, at a temperature of approximately 400° F. it produces a composition which upon cooling forms a gel.

In some instances the stearine pitch is quite acid and it is necessary to partially neutralize this pitch in order to obtain a satisfactory gel during preparation with most metallic soaps. However, I have discovered that acidity is of little importance in the production of gels from 35 stearine pitch with aluminium palmitate. Stearine pitch which is too acidic to produce gels with aluminium stearate, readily gels with aluminium palmitate.

These gels are extremely tough and elastic and 40 possess considerable elasticity even when cooled to a low temperature. The softening point of this gel may be varied over an appreciably wide range by varying the quantity of metallic soap used.

45 Other materials, such as asphalt or coal tar, may be substituted for part or all of the stearine pitch. Furthermore I may also employ pitches formed during the manufacture of oleic, palmitic, lauric, or other fatty acids, and when I employ 50 the term "pitch" in the specification and claims, it will be understood to embrace any or all of the foregoing materials. Furthermore, while aluminium palmitate is found to be a very satisfactory metallic soap for the preparation of the 55 gel with the stearine pitch, I find that other metallic soaps are capable of producing satisfactory gels with stearine pitch. For example, I may also employ iron stearate, iron palmitate, iron laurate, aluminium stearate, aluminium 60 laurate or aluminium naphthenate in the place of aluminium palmitate for the production of the gel with stearine pitch, coal tar, asphalt, or other pitches described above. Moreover, a metallic soap of zinc, calcium, magnesium or other 65 metal may be substituted for all or part of the aluminium palmitate.

The gels produced by the combination of 70 pitches with the foregoing metallic soaps may be compounded with various materials, such as waxes, wax gels, synthetic waxes, mineral fillers such as talc or clay, natural or synthetic resins, organic fillers such as starch, perfumes, water, glycerines, glycols, graphite, or lubricants for the production of a large number of plastic 75 compositions suitable for use in the dental art

and elsewhere where impressions, casts or models are employed. For example, compositions may be formulated suitable for the reproduction of facial or other anatomical features, or for the duplication of models, etc.

It is, therefore, an object of my invention to produce gels from metallic soaps and pitches.

It is a further object of my invention to produce gels by combining stearine pitch with a metallic soap, such as aluminium palmitate.

10 It is a further object of my invention to produce impression compositions by compounding gels produced from pitches and metallic soaps with fillers, waxes, resins, water, polyhydric alcohols, graphite or oils or mixtures thereof.

15 It is a further object of my invention to produce impression compositions by compounding gels produced from stearine pitch and aluminium palmitate with fillers, waxes, resins, water polyhydric alcohols, graphite or oils or mixtures 20 thereof.

It is a further object of my invention to produce impression compositions so compounded that they become elastic gels at or slightly above 98.6° F., and thus require no special cooling in 25 order to obtain the proper degree of rigidity when used for dental impression purposes.

These gels and especially the gel produced from stearine pitch and metallic soaps are highly 30 satisfactory as bases to be compounded with other materials as I have previously described.

In the preparation of the gel from stearine pitch and aluminium palmitate I proceed as follows:

15 pounds of stearine pitch are melted in a 35 kettle over an open flame and the temperature raised to approximately 350° F. 7 pounds of aluminium palmitate are then added and the mixture agitated while the temperature is raised to approximately 400° F., and heating and agitation 40 continued until a smooth viscous mass is obtained which on cooling sets to a firm gel.

The firmness and softening point of this gel may be modified by using more or less of the metallic soap, or by the addition of plasticizers 45 such as fatty acids, rosin, abietic acid, waxes, etc. It is also possible to add resins or waxes of high melting point, such as synthetic wax to increase the firmness of the gel when cooled.

An example of a composition which I have 50 found to be highly satisfactory for making dental impressions and which contains stearine pitch gelled with a metallic soap is as follows:

|                                                                | Pounds | 55 |
|----------------------------------------------------------------|--------|----|
| Stearine pitch, M. P. 150° F.                                  | 90     |    |
| Stearic acid                                                   | 13     |    |
| Latex                                                          | 15     |    |
| Aluminum palmitate                                             | 35     |    |
| Gel of 60 parts Japan wax and 40 parts alu-<br>minum palmitate | 30     | 60 |
| Talc, 200 mesh or finer                                        | 36     |    |
| Water                                                          | 15     |    |

In making this composition, the stearine pitch and stearic acid are melted together and brought 65 to a temperature of approximately 350° F., the addition of stearic acid making the melt more fluid and serving later to plasticize the gel. The latex is then added and the heat maintained with agitation until the water from the latex has 70 evaporated and the rubber all gone into smooth solution, this serving later to toughen the gel. The aluminium palmitate is then added and the temperature increased to approximately 400° F., and agitation maintained until a smooth mixture 75

is obtained which on cooling becomes a stiff gel. The mixture is then allowed to cool to approximately 200° F. and the Japan wax gel, which has been previously prepared by heating 60 parts of Japan wax with 40 parts of aluminum palmitate at approximately 350° F. until homogeneous and cooling, is added, together with the talc and water, and the whole thoroughly mixed.

The addition of the Japan wax gel lengthens the period of change from the plastic to the elastic gel, and makes easier the incorporation of the water in an emulsified condition, which in turn plasticizes the composition and makes it more adapted to flow under pressure when warmed and thus fill all the recesses, crevices and other irregularities in the teeth and gums when pressed into engagement therewith. The addition of talc adds smoothness to the compound and increases its specific gravity so that it can be made floating or non-floating as desired. The proportion of aluminium palmitate may be varied to some extent with different lots of stearine pitch. Too small an amount produces a gel which is too soft and somewhat sticky, and too large an amount produces a stiff gel which is not readily plasticized. If desired, from 3 to 10 pounds of rosin or of a solution of shellac melted in rosin may be added to increase the adherence of the material to itself, and it is also possible to add small amounts of lubricating agents, such as glycerine, graphite or aluminium powder if desired for any particular purpose, and also to add stiffening agents, such as synthetic wax having a melting point above 100° C. to render the material harder when cold and more easily removed from plaster cast into an impression taken with this composition.

A further example of a composition which I have found to be highly satisfactory for making dental impressions and which contains stearine pitch gelled with a metallic soap is as follows:

|                                                       | Pounds |
|-------------------------------------------------------|--------|
| Stearine pitch (melting point) 150° F.                | 90     |
| Synthetic wax having a melting point above 45 100° C. | 19     |
| Aluminium palmitate                                   | 40     |
| Rosin                                                 | 7      |
| Talc                                                  | 10     |
| Water                                                 | 5      |

In making this composition, the stearine pitch and synthetic wax are melted together, the aluminium palmitate added, and the temperature increased to approximately 400° F. and agitation maintained until a smooth mixture is obtained which on cooling becomes a stiff gel. The mixture is then allowed to cool to approximately 200° F. and the rosin added, and when this has dissolved and the mixture been agitated until smooth, the talc and water are added and the whole thoroughly mixed.

In this composition, the synthetic wax softens the mixture when warm and renders it harder when cold, while the rosin plasticizes the stearine pitch-metallic soap gel and aids the emulsification of the water which also plasticizes the composition. The talc adds smoothness and weight.

The above compositions are adapted to become plastic within a temperature range comfortable to the mouth, i. e., between approximately 100°-140° F. In using them, the dentist usually places in water a portion of the composition of suitable size for the impression to be taken, and warms the water until the material is plastic enough to knead smooth with the fingers and be shaped into the impression tray or other appliance to be used. He then loads the tray or appliance suitably with the plastic material, seats it to place in the mouth, compressing the material so as to force it into the crevices, undercuts and irregularities of the teeth and gums, and holds the tray without permitting movement while the impression material 15 cools from the plastic to the elastic gel state, usually requiring two to five minutes contact with the mouth if no cooling water or cold air is used to aid chilling. The tray containing the impression may then be removed from the mouth, cooled 20 further if desired to additionally stiffen the impression material, and used as a mold for casting plaster of Paris or in any other way desired. Care is taken not to cool the material too far before removal from the mouth, as if too cold, the 25 elastic gel state may be passed and the material becomes so rigid that permanent distortion may occur during removal.

It is obvious that by varying the proportions and ingredients mentioned, the properties of the composition may be altered over a considerable range, and I do not wish to be limited by the examples given, as they are merely illustrative of the invention which I claim.

I claim:

1. An impression material comprising a fatty acid pitch jelled with a metallic soap. 35
2. An impression material comprising a fatty acid pitch jelled with a metallic soap of palmitic acid. 40
3. An impression material comprising stearine pitch gelled with a metallic soap. 45
4. An impression material comprising stearine pitch gelled with a metallic soap of palmitic acid. 50
5. An impression material comprising stearine pitch gelled with aluminium palmitate. 55
6. An impression material comprising stearine pitch, synthetic wax having a melting point above 100° C., aluminium palmitate, a mineral filler and water. 60
7. An impression material comprising approximately 90 parts of stearine pitch, 19 parts of synthetic wax having a melting point above 100° C., 40 parts of aluminium palmitate, 10 parts of a mineral filler, and 1 part of water. 65
8. An impression material comprising stearine pitch, synthetic wax having a melting point above 100° C., aluminium palmitate, rosin, a mineral filler and water. 70
9. An impression material comprising 90 parts of stearine pitch, 19 parts of synthetic wax having a melting point above 100° C., 40 parts of aluminium palmitate, 7 parts of rosin, 10 parts of talc and 5 parts of water. 75

RAYMOND B. STRINGFIELD.